# EUROPEAN PATENT SPECIFICATION

(11) **EP 1 306 142 B1**
(45) Date of publication and mention of the grant of the patent: **30.08.2006**
(21) Application number: 01957647.9
(22) Date of filing: 29.06.2001
(51) Int. Cl.: B21B 1/02

(54) **METHOD FOR SEPARATING ROLLING OF STOCK MATERIAL**
VERFAHREN ZUM LÄNGSTRENNWALZEN VON WALZGUT
PROCEDE DE LAMINAGE DE FLANS PAR SEPARATION

(30) Priority: 04.07.2000 BY 20000637; 12.12.2000 RU 2000125597
(43) Date of publication of application: 02.05.2003
(73) Proprietor: Respublikanskoe Unitarnoe Predpriyatie "Belorussky Metallurgichesky Zavod", Gomelskaya obl., 247210 (BY)
(72) Inventor: BONDARENKO, Alexandr Nickolaevich, Gomelskaya obl., 247210 (BY); PHILIPPOV, Vadim Vladimirovich, Gomelskaya obl., 247210 (BY); GULYAEV, Michail Pavlovich, Gomelskaya obl., 247210 (BY); DYACHENKO, Yuri Vladimirovich, Gomelskaya obl., 247210 (BY); TISCHENKO, Vladimir Andreevich, Gomelskaya obl., 247210 (BY)
(74) Representative: Lins, Edgar
(86) International application number: PCT/BY2001/000009
(87) International publication number: WO 2002/002250

(56) References cited:
- GB-A- 191 128 777
- RU-C1- 2 126 728
- SU-A- 1 061 860
- US-A- 6 050 122
- DATABASE WPI Section Ch, Week 199402 Derwent Publications Ltd., London, GB; Class M21, AN 1994-015278 XP002342307 -& SU 1 784 293 A1 (FERROUS METALLURGY INST) 30 December 1992 (1992-12-30)
- SHUBIN S G ET AL: "INVESTIGATION OF THE TECHNOLOGICAL POSSIBILITIES OF THE PROCESS OF MULTISTRAND ROLLING AND SEPARATING ROUNDS" STEEL IN TRANSLATION, INSTITUTE OF MATERIALS, LONDON, GB, vol. 29, no. 8, 1999, pages 55-58, XP000976460 ISSN: 0967-0912
- DATABASE WPI Section Ch, Week 197926 Derwent Publications Ltd., London, GB; Class M21, AN 1979-48746B XP002342308 -& SU 622 514 A (DONETSK POLY) 22 July 1978 (1978-07-22)

## Description

### Field of the invention

The present invention relates to rolling process, particularly to the methods of rolling at reversing mills, roughing mills, continuous billet mills and heavy section mills chiefly for billet production.

### Description of the prior art

The following methods are already known: billet rolling at roughing and billet mills by means of successively arranged box passes, a square box pass, rhombic and diagonal square passes.

The method of billet rolling at a reversing roughing mill [1] which includes applying of successive flat box passes with the groove bottom surface bent relative to its vertical axis towards the sidewalls situated on the body of the roll along its length, a square box pass with the groove sidewalls taper, a rhombic pass and a diagonal square pass was taken as a prototype.

The disadvantage of this method is the tendency of the feed coming from the rhombic pass to twist in the diagonal square pass which results in a worse quality of the finished product. This happens because the feed coming from the square box pass loses its diagonal symmetry during the operation (e.g. this may be caused by a wear of the pass). Due to this reason the feed coming from the rhombic pass loses its rhombic shape, i.e. the rhomb made in this pass loses its diagonal symmetry. When such feed goes through the diagonal square pass, it twists round its longitudinal axis and, besides the impairment of the quality of the finished product, this causes feed handling problems (e.g. manipulating, cross motion, etc.), it also makes the rolling cycle longer and lowers mill performance characteristics .

Other disadvantages of this rolling method are:
- Impossibility to improve the ingot macrostructure having internal melting defects concentrated in its core part (e.g. central porosity, carbon segregation);
- Worse quality of the finished product and lower mill performance characteristics caused by the feed coming from the rhombic pass tendency to twist in the diagonal square pass due to the loss of the feed diagonal symmetry while passing through the box passes during the operation (e.g. due to the pass wear);
- low production rate of the mill.

### Summary of the invention

The object of the present invention is to provide simultaneous double feed rolling in square passes, to improve finished product quality, particularly its macrostructure, giving a heavy reduction to ingot core part, to improve mill performance characteristics.

Technological effects of the present invention are elimination of the feed twisting round its longitudinal axis in the diagonal square passes, decrease of ingot macrostructure defects due to axial porosity compacting and complete elimination of carbon segregation.

The object of the present invention is achieved because in the slitting method of billet rolling according to which a heated feed is rolled successively in box, rhombic and diagonal square passes of the rolling mill, after the box pass a feed is rolled in a forming slitting pass having the shape of two ovals connected by a bridge and after that in rhombic and diagonal square passes it is further rolled into two feeds connected by a bridge, whereby double diagonal squares are slit in a breaking pass by means of round groove ridges having the radius R = (0,3...0,45)a, where a - a square billet side.

The difference between the method of the present invention and its prototype is that after the box pass the feed is rolled in the forming slitting pass having the shape of two ovals connected by a bridge and then in rhombic and diagonal square passes in the form of two grooves connected by a bridge, whereby the dual diagonal squares are slit in the breaking pass by means of round groove ridges having the radius R = (0,3...0,45)a, where a - a square billet side.

### Brief description of the drawings

The following drawings are given to illustrate the invention.

Fig. 1 illustrates a roll pass design consisting of five passes.

Fig.2 schematically represents the pass consisting of two diagonal squares connected by a bridge.

Fig.3 schematically represents a breaking pass, providing the bridge breaking and the double feed splitting into two separate billets.

### Preferable embodiments of the invention

The process of rolling using the system of passes according to the present invention is done as follows. The original ingot with square or rectangular cross-section is heated in the reheating furnace of a roughing mill and is rolled first in a box pass 1 with the groove bottom surface bent about the pass vertical axis. After the box pass the feed is rolled in a forming (slitting) pass 2 having the shape of a twin feed, both parts of which have similar sectional areas of an oval or rhombic shape connected by a bridge. In the process of deformation in pass 2 incoming rectangular feed centers itself in the pass at the moment of nipping due to simultaneous four - angle contact with the sidewalls of the pass and after slitting by means of the pass grooves ridges situated on the central vertical axis of the pass, two feeds with the same cross-section connected by a bridge are formed. The following feed forming is carried out in two passes representing double passes with rhombic (pass 3) and rectangular (pass 4) cross-sections connected by bridges, where deformation occurs in a rhombic - square roll pass design without twisting round the longitudinal axis as distinct from the previously known rhomb - square pass design method (1).

The rolling method of the invention allows a greater degree of deformation of the original ingot core part where casting defects - central porosity and carbon segregation - are concentrated. For instance, diagonal square height total reduction coefficient in pass 4 is 1.8, and bridge total reduction coefficient in this pass is 75. High degree of the feed core part deformation allows to eliminate the original ingot central porosity. Due to the rolling method of the invention carbon segregation (casting defect) moves to the bridge area connecting two diagonal squares (fig.2).

The double feed being rolled in pass 5 is slit into two square billets by means of slitting ridges having the radius R = (0,30-0,45)a, where "a" is square billet side (Fig.3), separating the double diagonal square to the distance 1₂ (fig.2), which is 1,1 - 1,3 times as long as the distance 1₁.

Separated square billets having remains of the bridge at the point of slitting are dressed with a grinding machine removing bridge remains where carbon segregation is concentrated.

### Industrial application

The method of the invention is implemented at a roughing two-high reversing rolling mill 850 at the Republican Unitary Enterprise "Byelorussian Steel Works" in manufacturing of high carbon steel st80 cord square billet 125x125 mm used for cord rod production.

The original ingot with square or rectangular cross-section is heated in the heating furnace of a roughing mill and is rolled first in a box pass 1 with the groove bottom surface bent about the pass standing axis. After the box pass the feed is rolled in a forming (slitting) pass 2 having the shape of double feed, both parts of which have the same sectional areas of an oval or rhombic shape connected by a bridge. In the process of deformation in pass 2 the incoming rectangular feed centers itself in the pass at the moment of nipping due to simultaneous four-angle contact with the sidewalls of the pass and after slitting by means of the pass grooves ridges situated on the central vertical axis of the pass, two feeds with the same cross-section connected by a bridge are formed. The following feed formation is carried out in two passes representing double passes with rhombic (pass 3) and rectangular (pass 4) cross-sections connected by bridges, where deformation occurs without twisting round the longitudinal axis as distinct from the previously known rhomb-square pass design method.

The double feed being rolled in pass 5 is slit into two square billets by means of slitting ridges having the radius R = (0,30-0,45)a, where "a" - a square billet side (Fig.3), separating double diagonal squares to the distance 1₂ (fig.2), which is 1,1 - 1,3 times as long as the distance 1₁.

Separated square billets having bridge remains at the point of slitting are dressed with a grinding machine, thus, bridge remains where segregation is carbon concentrated are removed.

The method of the invention implemented under the conditions of the roughing rolling mill 850 allows to eliminate diagonal square twisting round the longitudinal axis, to improve mill performance characteristics due to simultaneous two square billets 125x125 mm rolling in the last pass and improve the billet macrostructure quality due to axial porosity compacting and complete elimination of carbon segregation.

### Source of information

1. Filippov I.N. and others. Roll pass designs atlas. - M.: Chermetinformatsiya, 1965. - pp. 11 - 12 (prototype).

## Claims

1. A method of billet rolling in which heated ingot is rolled successively in box, rhombic and diagonal square passes of a rolling mill **characterized by** rolling of a billet in a box pass, then in a forming slitting pass having the shape of two ovals connected by a bridge and after that in rhombic and diagonal square passes where it is further rolled into two feeds connected by a bridge, where the double diagonal squares being slit in a succeeding breaking pass by means of round groove ridges having the radius R = (0,3...0,45)a, where "a" is a square billet side.

## Patentansprüche

1. Verfahren zum Walzen von Knüppeln, bei dem ein aufgeheizter Block nacheinander in Kasten-, Rhombus- und quadratischen Diagonalstichen einer Walzstraße gewalzt wird, **gekennzeichnet durch** das Walzen eines Knüppels in einem Kastenstich, anschließend in einem formgebenden Schlitzwalzstich in Form von zwei durch eine Brücke verbundenen Ovalen und danach in Rhombus- und quadratischen Diagonalstichen, wo das Walzen in zwei **durch** eine Brücke verbundenen Strängen erfolgt, wobei die doppelten diagonalen Quadrate in einem nachfolgenden Trennstich mit runden Kaliberstegen mit einem Radius R = (0,3...0,45) a geschnitten werden, wobei "a" die Kantenlänge des quadratischen Knüppels ist.

## Revendications

1. Procédé de laminage de billettes dans lequel un lingot chauffé est successivement laminé dans des cannelures de roulage, losanges, et carrées diagonales d'un laminoir, **caractérisé par** le laminage d'une billette dans une cannelure de roulage, puis dans une cannelure pour former et fendre ayant la forme de deux ovales reliés par un pont, puis dans des cannelures losanges et carrées diagonales où elle est encore laminée en deux blocs reliés par un pont, procédé dans lequel le double carré est fendu dans une cannelure de cassage qui suit, au moyen de crêtes de gorge arrondies ayant un rayon R=(0,3...0,45)a, où « a » est le côté d'une billette carrée.
